

Patented Nov. 6, 1945

2,388,400

## UNITED STATES PATENT OFFICE

2,388,400

VANADIUM SALTS OF ACID ESTERS AS  
INHIBITORS IN LUBRICATING OILS

Frederick C. Frank, Pitman, and Darwin E. Badertscher and Henry G. Berger, Woodbury, N. J., assignors to Socony-Vacuum Oil Company, Incorporated, New York, N. Y., a corporation of New York

No Drawing. Application March 17, 1942,  
Serial No. 435,082

2 Claims. (Cl. 252—35)

This invention has to do in a general way with mineral oil compositions and is more particularly concerned with the production of mineral oil fractions of the viscous type, such as are used for lubricants, dielectrics, etc., which have been improved by the incorporation therein of a minor proportion of an oil-miscible metal organic compound capable of inhibiting the deleterious effects of oxidation upon the oil.

As is well known to those familiar with the art, the ordinary lubricating oils such, for example, as are used in the lubrication of internal combustion engines, will, as the result of oxidation under normal conditions of use, develop substantial quantities of carbonaceous deposits which accumulate as sludge or "carbon deposits" impairing the free flow of the oil, and which deposit about the piston rings, causing them to stick and filling the slots in the oil rings. There is also developed, as the result of oxidation, substantial acidity in the oil which has a deleterious effect upon contacted metals, particularly certain types of alloy bearing metals; and in the event the oil is being used as a dielectric, the development of acidity obviously reduces its efficiency in this respect.

Numerous additive agents or "oxidation inhibitors" have been developed for use in mineral oils to retard or counteract the effects of oxidation. In general, the more effective of these oxidation inhibitors when incorporated in mineral oil fractions will inhibit the effects of oxidation upon the oil for a limited time; and when the oil composition is removed from the engine in which it has been used and is substituted by a mineral oil fraction which does not contain an oxidation inhibitor, the oil will deteriorate during use. Thus, there is no carrying over of the effect of the inhibited mineral oil to a blank mineral oil used in a succeeding engine operation.

The present invention is predicated upon our discovery of a novel class of oxidation inhibitors and is broadly directed to viscous mineral oil compositions which have been inhibited against oxidation by the incorporation therein of one or more compounds or compositions belonging to this general class. The improving agents contemplated herein as oxidation inhibitors belong to the general class of metal salts or soaps of organic acids. More specifically, the present invention is predicated upon the discovery that the vanadium salts of certain types of organic acids possess unique properties as lubricating oil addition agents. Broadly stated the compounds contemplated herein are the vanadium salts of acid esters of

polycarboxylic acids in which the hydrogen of one carboxyl group has been replaced with an alicyclic or aliphatic hydrocarbon group containing a sufficient number of carbon atoms or an aliphatic group of sufficiently high "molecular weight" to solubilize the compound in viscous mineral oil; and particularly preferred for the purposes of the present invention are the corresponding vanadyl salts.

10 Compounds of this general class of vanadium salts or soaps, particularly the vanadyl salts or soaps, are not only extremely effective as oxidation inhibitors when used in internal combustion engines, but they also possess the surprising property of conditioning the engine parts in some way, so that when the inhibited oil is removed from the engine in which it has been used and an uninhibited oil subsequently used in the engine, the uninhibited oil will not undergo the deterioration which would normally be encountered in such use. This remarkable property is not fleeting nor limited to one following engine run, but continues in effect for a number of such subsequent engine operations. In effect, we have discovered that by 15 lubricating an engine—as, an internal combustion engine—with a mineral oil containing one or more of our novel vanadium-organic compounds, as vanadyl-organic compounds, uninhibited mineral oils subsequently used in the engine 20 will be, in fact, inhibited by some as yet unexplained action of the additive.

The aforesaid conditioning action appears to be critical with vanadium salts—as typified by the vanadyl salts—of the acid esters described 25 above, for the corresponding salts of other polyvalent metals do not act in the same manner as do the vanadium salts. Results of the Accelerated ring sticking test given hereinafter in Table III of typical polyvalent metal salts indicate that 30 only the vanadium compounds are capable of imparting this surprising conditioning effect to the engine.

The acid esters, from which the salts contemplated herein are obtained, can be formed by the 35 reaction of aliphatic or alicyclic alcohols with an aliphatic, cycloaliphatic or aromatic polycarboxylic acid. Typical polycarboxylic acids which may be used are maleic, succinic, malonic, phthalic, etc. The vanadium salts may be formed by first 40 neutralizing the acid with an alkali alcoholate or alkali metal hydroxide to form the alkali metal salt and then effecting a so-called "metathesis" with an inorganic vanadium salt.

In the case of acid ester salts derived from the 45 dicarboxylic acids, which have been used to dem-

onstrate the effectiveness of the compounds contemplated herein, these compounds may be represented by the general formula:



in which  $\text{R}'$  represents the mineral oil-solubilizing aliphatic or alicyclic group which we have discovered should contain at least three carbon atoms to give the desired property of oil-miscibility in the product;  $x$  represents a whole number which may be 2, 3, 4 or 5; and the group



may be described as representing the residue of an aliphatic, alicyclic, or aromatic dicarboxylic acid. In certain of the compounds synthesized to demonstrate the effectiveness of this class of materials as oxidation inhibitors,  $\text{R}$  may be considered as broadly representing a mono or polycyclic aromatic nucleus and preferably a phenylene group, the group



being the residue of phthalic acid, in which  $\text{R}$  is  $\text{C}_6\text{H}_4$ . In the foregoing general formula I, the symbol  $\text{V}'$  is used to represent both the element vanadium and the vanadyl ( $\text{V}=\text{O}$ ) group. Also, where the term "vanadium salt" is used herein, such term is employed in the broad sense and is inclusive of the true vanadium salts, vanadyl salts and the like.

Particularly preferred, however, for the purposes of the present invention are the vanadyl salts of the acid esters hereinbefore described, which are represented by the following general formula:



in which  $\text{R}$  and  $\text{R}'$  are as given above.

From the foregoing it will be seen that the compounds contemplated herein as oil-improving agents may be broadly classified as the vanadium salts of an acid ester of a polycarboxylic acid wherein the hydrogen of at least one carboxyl group is replaced with an aliphatic or alicyclic group having at least 3 carbon atoms.

The synthesis of salts of the type contemplated by this invention is illustrated by the following description of the procedure followed in preparing vanadyl oleyl-phthalate.

#### EXAMPLE I

Vanadyl oleyl phthalate was prepared in three separate stages:

##### (a) HYDROGEN OLEYL PHTHALATE

A mixture of 268 grams (1 mole) of commercial oleyl alcohol, 268 grams (1.8 moles) of phthalic anhydride and 1000 c. c. of benzene was distilled until 400 c. c. of benzene had been removed (to make the mixture anhydrous). The distillation residue was then stirred and refluxed on a hot water bath for 7.25 hours. After cooling over night the mixture was filtered off by suction. The unreacted phthalic anhydride from this filtration weighed 95 grams. The filtrate was vacuum distilled on the water bath to remove the benzene. The cold distillation residue which had deposited more phthalic anhydride, was filtered

and the phthalic anhydride washed in the filter with petroleum ether. The phthalic anhydride thus recovered weighed 27 grams. The petroleum ether was evaporated and the residue combined with the main bulk of the product. The total recovery of unreacted phthalic anhydride was 122 grams (theoretical recovery, 120 grams). The total yield of product with a neutralization number of 138.0 (theoretical, 139.3) was 395 grams, 95% of that required by theory.

##### (b) SODIUM OLEYL PHTHALATE

To a solution of sodium ethylate prepared from 5.5 grams of metallic sodium and 75 cc. absolute alcohol was added with stirring a solution of 100 grams hydrogen oleyl phthalate in 200 cc. petroleum ether. Removal of the alcohol and petroleum ether by vacuum distillation on the water bath yielded as a residue 100 grams of a solid, somewhat hygroscopic soap.

##### (c) VANADYL OLEYL PHTHALATE

To a solution of sodium oleyl phthalate prepared by the action of 7 grams of sodium and 25 cc. absolute alcohol on a solution of 127 grams of hydrogen oleyl phthalate in 250 cc. dry benzene, was added 28 grams of syrupy vanadyl chloride which is a hydrate, possibly



(Cf. Merck's Index). The mixture was refluxed with stirring in an apparatus with a water "take-off" so that the water in the vanadyl chloride was removed and the mixture made anhydrous. The mixture was then filtered free from sodium chloride and the benzene evaporated leaving 138 grams of a dark green, viscous liquid (theoretical yield 137.5 grams).

The vanadium salts, as typified by the vanadyl salts, contemplated by this invention are highly viscous products and are soluble in mineral oil when the aliphatic ester constituent is comprised of three or more carbon atoms. Other typical vanadyl salts contemplated by the present invention are vanadyl oleyl succinate, vanadyl oleyl malonate, vanadyl oleyl maleate, vanadyl oleyl tetrahydro phthalate, etc.

To demonstrate the effectiveness of the vanadium-organic salts contemplated by this invention as oxidation inhibitors for viscous mineral oils, we have subjected samples of an unblended oil and a blend of the same oil containing the improving agent to the Bubble test, which comprises the following. A section of bearing containing a cadmium-silver alloy surface and weighing about 6.0 grams was placed in 30 grams of a commercial S. A. E. 20 solvent-refined motor oil. The oil was heated to about 175° C. for 22 hours while a stream of air was bubbled against the surface of the bearing. The weight loss in milligrams of the bearing is interpreted as a measure of the corrosiveness of the oil. The inhibited and uninhibited oil samples were run concurrently, the results of which are given in Table I below.

Table I

| Sample                                              | Milligrams loss |
|-----------------------------------------------------|-----------------|
| Uninhibited oil                                     | 61              |
| Oil + 0.625% (by weight) of vanadyl oleyl phthalate | 8               |

To further demonstrate the effectiveness of the salts contemplated by this invention as oxidation inhibitors for viscous mineral oils, we have

subjected samples of an unblended solvent-refined S. A. E. 30 motor oil and a blend of the same oil containing our typical improving agent to an Oxidation susceptibility test. In this test, 300 gram samples of oil in pyrex glass beakers were maintained at 350° F. and 2 liters of air per hour were blown over the surface while the samples were stirred constantly with steel paddles. Samples were withdrawn at specified intervals and the volume-percentage of sludge determined. The results of this test are given below in Table II.

Table II

| Material added          | Wt. per cent | Sludge, volume percentage |        |        | 15 |
|-------------------------|--------------|---------------------------|--------|--------|----|
|                         |              | 3 days                    | 5 days | 7 days |    |
| None                    |              |                           |        | 12     |    |
| Vanadyl oleyl phthalate | 1.00         | 0.5                       | 0.5    | 1.0    | 20 |

The most impressive demonstration of the effectiveness of the salts contemplated by this in-

vention as oxidation inhibitors for viscous mineral oils is given by the results of the Accelerated ring sticking test. The engine employed in this test was the standard C. F. R. "Knock test" engine which is cooled with a diethylene glycol-water mixture held at about 400° F. The engine was run at a speed of approximately 1200 R. P. M. with the throttle set just below detonation, using a compression ratio of 7:1. The runs were normally for 28 hours, with an inspection of the piston at 14 hours. At the end of the test the piston was examined for stuck rings, ring slots filled with carbonaceous deposits and total deposits. The acidity or neutralization number (N.N.) of the used oil and the kinematic viscosity of the used oil were determined. The oil used was a lubricating oil stock of 120 seconds Saybolt Universal viscosity at 210° F. and the results of the consecutive engine runs are tabulated in Table III. After each engine run with an oil blend, at least one run was made with the fresh unblended oil to determine the "carry over" effect of the additive which was in the oil blend in question.

Table III

| Run No. | Additive                  | Percent by wt. | Hours | Rings, degrees stuck |     |     |     |     | Slots per cent filled |    |    | Total deposits | Used oil     |       |       |     |
|---------|---------------------------|----------------|-------|----------------------|-----|-----|-----|-----|-----------------------|----|----|----------------|--------------|-------|-------|-----|
|         |                           |                |       | 1                    | 2   | 3   | 4   | 5   | 3                     | 4  | 5  |                | 210° F. K.V. | N. N. |       |     |
| 1       | None                      |                | 14    | 0                    | 0   | 0   | 0   | 0   | 5                     | 5  | 0  | 10.6           | 30.14        | 2.0   |       |     |
| 2a      | Aluminum oleyl phthalate  | 1.0            | 14    | 330                  | 360 | 360 | 200 | 75  | 90                    | 20 | 0  | 5.8            | 31.12        | 2.5   |       |     |
| 2b      | None                      |                | 14    | 90                   | 0   | 0   | 0   | 0   | 0                     | 0  | 0  | 9.45           | 26.87        | 1.3   |       |     |
| 3a      | Barium oleyl phthalate    | 1.0            | 14    | 180                  | 0   | 0   | 0   | 0   | Tr                    | 0  | 0  | 7.35           | 30.60        | 3.0   |       |     |
| 3b      | None                      |                | 14    | 360                  | 360 | 0   | 0   | 25  | 40                    | Tr | 0  | 18.75          | 30.4         | 1.2   |       |     |
| 4a      | Cobaltous oleyl phthalate | 1.0            | 14    | 10                   | 0   | 0   | 0   | 0   | 0                     | 0  | 0  | 0              | 3.35         | 33.04 | 2.6   |     |
| 4b      | None                      |                | 14    | 150                  | 0   | 0   | 0   | 0   | 50                    | 15 | Tr | 0              | 12.93        | 29.60 | 2.3   |     |
| 5a      | Ferrous oleyl phthalate   | 1.0            | 14    | 280                  | 0   | 360 | 360 | 360 | 90                    | 85 | 20 | 10.1           | 26.58        | 1.7   |       |     |
| 5b      | None                      |                | 14    | 360                  | 0   | 360 | 360 | 360 | 70                    | 85 | 5  | 14.1           | 29.76        | 2.3   |       |     |
| 6a      | Manganous oleyl phthalate | 1.0            | 14    | 360                  | 0   | 0   | 0   | 0   | 0                     | 0  | 0  | 5.0            | 38.06        | 0.7   |       |     |
| 6b      | None                      |                | 14    | 360                  | 0   | 180 | T   | 0   | 50                    | 40 | 10 | 0              | 10.0         | 29.04 | 1.5   |     |
| 7a      | Stannous oleyl phthalate  | 1.0            | 14    | 30                   | 0   | 0   | 0   | 0   | 5                     | Tr | Tr | 0              | 6.0          | 29.40 | 2.2   |     |
| 7b      | None                      |                | 14    | 0                    | 0   | 360 | VT  | VT  | 75                    | 20 | 10 | 0              | 0            | 0     | 0     |     |
| 8a      | Vanadyl oleyl phthalate   | 1.0            | 14    | 220                  | 0   | 360 | 360 | 360 | 95                    | 90 | 85 | 16.8           | 28.55        | 1.7   |       |     |
| 8b      | None                      |                | 14    | 0                    | 0   | 0   | 0   | 0   | 0                     | 0  | 0  | 0              | 3.5          | 24.98 | 0.6   |     |
| 8c      | do                        |                | 14    | 0                    | 0   | 0   | 0   | 0   | 0                     | 0  | 0  | 0              | 6.4          | 26.18 | 0.5   |     |
| 8d      | do                        |                | 14    | 0                    | 0   | 0   | T   | 0   | 0                     | 0  | 5  | Tr             | 10.0         | 26.89 | 1.0   |     |
| 8e      | do                        |                | 14    | 0                    | 0   | 0   | 0   | 0   | 0                     | 0  | 0  | 0              | 16.9         | 27.66 | 2.5   |     |
| 8f      | do                        |                | 14    | 0                    | 0   | 0   | 0   | 0   | 15                    | 10 | Tr | 0              | 5.1          | 12.35 | 28.06 | 1.6 |
| 8g      | do                        |                | 14    | 360                  | 0   | 360 | 210 | 80  | 70                    | Tr | 0  | 0              | 14.1         | 29.76 | 2.3   |     |
| 9a      | Vanadyl oleyl phthalate   | 0.25           | 14    | 360                  | 0   | 360 | 360 | 360 | 0                     | 40 | 20 | 0              | 12.25        | 28.93 | 1.4   |     |
| 9b      | None                      |                | 14    | 0                    | 0   | 0   | 0   | 0   | 0                     | 0  | 0  | 0              | 5.65         | 26.05 | 0.5   |     |
| 9c      | do                        |                | 14    | 0                    | 0   | 0   | T   | T   | 20                    | 10 | Tr | 0              | 8.60         | 27.29 | 1.2   |     |
| 9d      | do                        |                | 14    | 0                    | 0   | 0   | 0   | 0   | 0                     | 0  | 0  | 0              | 12.25        | 28.28 | 1.1   |     |
|         |                           |                | 28    | 10                   | 360 | 360 | 360 | 360 | 75                    | 60 | 75 | 13.0           | 28.83        | 1.1   |       |     |

Tr—trace.

T—tacky.

VT—very tacky.

In the foregoing Table II where there are several engine runs designated by a single number (2a, 2b, or 8a, 8b, 8c, etc.), the data presented in connection with the same number was obtained from companion runs in that the run designated by the subscript "a" was made with a blend of the oil and the designated additive; and the next succeeding run, or runs, designated

70 by the same number and the subscription "b," or "c," etc., were made with fresh uninhibited oil without cleaning the engine after the blend of oil and additive had been removed. Prior to each initial "a" run with the oil blend containing the designated additive, the engine was thoroughly cleaned. These data were obtained to demonstrate the aforesaid "carry-over" effect of the

vanadium compounds, as illustrated by vanadyl compound, an effect not present in the corresponding compounds of the other metals tested. The vanadium compounds, particularly the vanadyl compounds, appear to be unique in this respect.

It will be observed, for example, that the results of engine runs 2a and 2b indicate that the incorporation of 1.0% of aluminum oleyl phthalate in the above-described oil improves the same, but when the fresh unblended oil is used in the succeeding engine run (2b) the improving effect is not present. In this particular run the performance with the "refill" was inferior to that with the same blank oil in the cleaning engine run (No. 1).

Similarly, the results of engine runs 3a-3b, 4a-4b, 5a-5b, 6a-6b, and 7a-7b indicate that the additives—in which the metal is other than vanadium—are effective for only the engine run in which the oil blend is used, and indicate also that the unblended oil is not improved by the use of the blended oil in a preceding engine run.

The results of engine runs 8a and 8b on the other hand demonstrate not only the effectiveness of the vanadium salt—as typified by a vanadyl salt—in the oil (as shown by 8a), but also the "carry-over" effect of the vanadium salt to the unblended oil in the succeeding engine run (as shown by 8b). Here it will be observed that the piston ring condition was the same with the refill oil at the end of 28 hours as it was with the blend (run 8a) whereas the blank oil in a clean engine (run No. 1) showed substantial ring sticking at the end of 28 hours. Further, the results of engine run 8b when compared with the results of the refill engine runs—2b, 3b, 4b, 5b, 6b and 7b—in which metal salts other than the vanadium salt had been used in prior engine runs, clearly show the superiority of the vanadium salt. It is also of interest to note that this "carry-over" effect obtains in gradually decreasing amounts after the first refill (8b) as evidenced by runs 8c, 8d and 8e, which is a surprising and unexpected result in the light of the other metals where the "carry-over" on the first refill, if present at all, is negligible.

Results of engine run 9a clearly indicate the efficacy of only 0.25% of the vanadium salt in the oil; and when the same results are compared

with any of the foregoing in which 1.0% of salts of other metals were used, it is readily seen that the smaller amount of the vanadium salt is much more effective than the larger amount of the salts of other metals, as, for example, Al, Ba, Co, Fe, Mn and Sn.

Thus, from the foregoing results, it will be seen that the vanadium—and particularly the vanadyl—ester acid salts of the type contemplated by this invention, when blended with a viscous mineral oil, retard to a substantial degree the deleterious effects of oxidation. The results of the Accelerated ring sticking test are particularly striking for they indicate that the vanadium salts as described herein are unique in imparting the above-described conditioning effect to engine parts, an effect not characteristic of corresponding salts of other poly-valent metals.

Improving agents of the type described above may be blended with mineral oil fractions in various proportions depending upon the oil fraction and the conditions under which it is used. In general, a satisfactory product may be obtained with about  $\frac{1}{4}\%$  of the improving agents, but amounts ranging from  $\frac{1}{16}\%$  to 2% may be used.

Our invention is not limited to the specific examples given herein but includes within its scope whatever changes or modifications fairly come within the spirit of the appended claims.

We claim:

1. A mineral oil composition comprising a viscous mineral oil fraction and in admixture therewith a minor proportion, sufficient to inhibit oxidation, of vanadyl oleyl phthalate, said phthalate having the property of inhibiting ring-sticking of pistons even after it is removed and the pistons are contacted with a compounded or non-compounded mineral oil.

2. A mineral oil composition comprising a viscous mineral oil fraction and in admixture therewith a minor proportion, from about  $\frac{1}{16}\%$  to about 2%, of vanadyl oleyl phthalate, said phthalate having the property of inhibiting ring-sticking of pistons even after it is removed and the pistons are contacted with a compounded or non-compounded mineral oil.

FREDERICK C. FRANK.

DARWIN E. BADERTSCHER.

HENRY G. BERGER.